

Sept. 28, 1965

R. F. CREW

3,208,920

PROCESS FOR ELECTROLYTICALLY DEPOSITING METALLIC MATERIAL

Filed Aug. 9, 1962



Inventor  
Richard F. Crew

By *[Signature]*

His Attorney

1

3,208,920

**PROCESS FOR ELECTROLYTICALLY DEPOSITING METALLIC MATERIAL**

Richard F. Crew, Alma, Mich., assignor to General Electric Company, a corporation of New York  
Filed Aug. 9, 1962, Ser. No. 215,849  
4 Claims. (Cl. 204—10)

This invention relates to an improved process for the preparation of metallic material by the electrolytic deposition of the metallic material into a liquid metal cathode.

Magnetic materials comprising elongated, single domain particles of improved magnetic properties may be obtained by the electrolytic deposition of fine metal magnetic particles into a pool of a liquid metal cathode, usually mercury. Such magnetic materials and their process of preparation are disclosed in U.S. Patent 2,974,104, which issued on March 7, 1961, and is assigned to the same assignee as the present invention.

During such electrodeposition, undesirable plating of the fine particles may occur on the tray on which the mercury is retained and on other portions of the cathode assembly. This interrupts and shortens the deposition cycle, requiring frequent removal of the components of the cathode assembly for cleaning and decreases the usable life span of such components.

Various methods for avoiding such plating on the cathode assembly components have proved unsuccessful. Decrease of current density, shortening of the plating cycle, use of special detergents in the electrolyte or the coating of the trays or other components of the cathode assembly with various non-conductive, organic materials either does not avoid the undesirable plating or results in degradation of the magnetic properties of the particles.

It is a primary object of this invention to provide a process for the electrodeposition of metallic material which avoids to a substantial extent undesirable plating of the metal on the various components of the liquid metal cathode assembly. It is an additional object of this invention to avoid such undesirable plating without adversely affecting either the deposition process or the properties of the particles deposited.

It has now been found that the foregoing and other objects of this invention may be achieved by coating the surfaces of the liquid metal cathode assembly with a polysiloxane fluid. The polysiloxane fluid does not affect the conductivity of the anode, cathode or electrolyte nor does it adversely affect the quality of the plated material. The polysiloxane coating sufficiently inhibits plating on the cathode assembly components to permit an increase of over twofold in the length of time for a given plating cycle and results in substantially reduced labor time involved in removing, cleaning and replacing the cathode assembly components. The invention is particularly useful in the preparation of elongated single domain magnetic particles prepared in accordance with the teachings of the above-mentioned U.S. Patent 2,974,104.

The term "cathode container assembly" as used herein means electrically insulated components of the electrolytic apparatus either in contact with, or in close proximity to, the liquid metal cathode. Such components ordinarily include the tray or other retaining surface for the cathode, structural members for supporting or suspending the tray, cathode leads and other components in association with the cathode, such as devices for feeding the liquid cathode into the tray. All of these components are either composed entirely of, or coated with, organic or inorganic electrically insulating materials such as glass, polyvinyl chloride, polyethylene, polystyrene, polyesters or other non-conductive materials well known in the art.

The invention will be more clearly understood by reference to the following description taken in connection

2

with the accompanying drawing in which the single figure illustrates in cross section an electrodeposition apparatus of the type with which the process of the present invention is useful.

5 A typical electrodeposition process involves the electrodeposition of particles of ferromagnetic material into a mercury cathode from an acidic electrolyte comprising ions of the ferromagnetic material, preferably while maintaining a quiescent interface between the cathode and the electrolyte. The electrolyte or plating solution may consist of the soluble salts of the ferromagnetic metals in the form of, for example, sulfates or chlorides. The pH of the electrolyte is made acidic with, for example, sulfuric or hydrochloric acid, a preferred pH being about 2. A 10 consumable anode is used of either the pure ferromagnetic metal or alloys of several ferromagnetic metals. A non-consumable anode of an inert material, such as graphite, may also be used. A current density between 5 and 100 amps/sq. ft. may be used. The electrolyte may be at 15 room temperature of 20 to 30° C. during electrodeposition, although other electrolyte temperatures may be used if suitable adjustments are made in current density and time of deposition. The foregoing process is more fully disclosed in the above-identified U.S. Patent 2,974,104 and 20 in copending application S.N. 161,033, filed December 21, 1961, and assigned to the same assignee as the present invention.

25 The drawing, illustrating an electrodeposition apparatus for carrying out the above process, shows an electroplating cell 1, including a glass tank 2, two vertically-suspended, consumable iron anodes 3, an electrolyte 4 consisting of an aqueous solution of ferrous sulfate, and a tray 5 in which is contained the mercury cathode 6. The tray 5 is suspended in the electrolyte from insulated suspension rods 7 connected to a cross support 8 resting on tank 2. Anode lead 9 and cathode lead 10 are connected to the positive and negative terminals, respectively, of a suitable D.C. source.

30 In accordance with the practice of this invention, the tray 5, the suspension rods 7 and the lead 10 are coated with a polysiloxane fluid before electrodeposition is begun. It is preferable to coat all surfaces of the cathode assembly within the tank 2 with the polysiloxane fluid although 35 it has been found that undesirable plating occurs largely on those surfaces in closest proximity to the surface of the liquid metal cathode. It may therefore be sufficient to coat only those portions of the cathode assembly on which such plating occurs.

35 The polysiloxane fluids which are useful in the practice of the present invention are liquid organopolysiloxane linear or branch chain compounds of the type disclosed in U.S. Patent 2,469,888 which issued on May 10, 1949 and is assigned to the assignee of the present invention. As there described, these organopolysiloxane chain compounds have the general formula



40 in which the various R's represent the same or different lower monovalent hydrocarbon radicals selected from the class consisting of lower alkyl, aryl, alkaryl, and aralkyl radicals, examples of which are the methyl, ethyl, propyl, phenyl, benzyl, tolyl and xylyl radicals and a is a whole number equal to at least 3. A preferred class of polysiloxane fluids are the trimethyl silyl chain-stopped methyl polysiloxanes of the formula



45 where n is a positive integer.

50 The invention is illustrated by the following examples.

*Example 1*

This example illustrates a deposition process for elongated, single domain iron particles using normal deposition current.

Iron particles were deposited using an electrolyte of ferrous sulfate of 1.52 molarity, two vertically-suspended iron anodes and a mercury cathode retained on a plastic tray of polyvinyl chloride. Portions of the tray, of the suspension rods and of the cathode lead adjacent to the mercury cathode, were coated with a trimethyl silyl chain-stopped dimethylpolysiloxane having a viscosity of 350 centistokes at 25° C. Other portions of the cathode assembly components adjacent to the mercury were left uncoated. The pH of the electrolyte was 2.0. Electrodeposition proceeded at a current density of 25 amps/sq. ft. for a time of 1 hour. The electrolyte was at room temperature.

At the conclusion of the electroplating cycle, the coated portions of the tray, cathode lead and cathode suspension rods, were observed to be free of undesirable deposition. The uncoated surfaces of the cathode assembly contained undesirable electroplated material.

*Example 2*

The electrodeposition process of Example 1 was repeated except that the current density was increased to 219 amps/sq. ft., almost nine times the current density normally used for electrodeposition of fine magnetic particles. For the duration of the electrodeposition cycle, the polysiloxane covered surfaces were free of deposited particles, whereas uncoated cathode assembly surfaces became plated.

Tests were made to determine the effect of the polysiloxane coating on the magnetic quality of the deposited particles. No degradation of properties was observed. Moreover, plating cycles—the duration for which the cell assembly may be continuously used without cleaning—were extended approximately two and one-half times with a considerable reduction in man-hours spent for inspection and cleaning of the cell assemblies.

The magnetic particles which may be deposited in accordance with the preferred embodiment of the invention may be any ferromagnetic metal or alloy such as, for example, iron, nickel, cobalt or alloys of iron, nickel and cobalt with each other or with other metals. While the invention has been particularly described in connection with the electrodeposition of elongated, single domain magnetic particles, it may be used in connection with

other electrodeposition methods to prevent undesirable plating on the cathode assembly.

What I claim as new and desire to secure by Letters Patent of the United States is:

- 5 1. A process comprising electrolytically depositing metallic material from an electrolyte comprising metallic ions of the material into a liquid metal cathode, said process being carried out in an electrolytic cell which includes a cathode container assembly of electrically insulating material for supporting said liquid metal cathode, said cathode container assembly being coated with a polysiloxane fluid.
- 10 2. A process comprising electrolytically depositing fine particle ferromagnetic material from an electrolyte comprising metallic ions of the ferromagnetic material into a mercury cathode, said process being carried out in an electrolytic cell which includes a cathode container assembly of electrically insulating material for supporting said liquid metal cathode, said cathode container assembly being coated with a polysiloxane fluid.
- 15 3. The process of claim 2 in which said polysiloxane fluid is a trimethyl silyl chain-stopped methyl polysiloxane.
- 20 4. A process comprising electrolytically depositing fine particle ferromagnetic material selected from the group consisting of iron, cobalt and nickel and alloys of iron, cobalt and nickel, from an electrolyte comprising metallic ions of the magnetic material into a mercury cathode while maintaining a quiescent interface between the cathode and electrolyte, said process being carried out in an electrolytic cell which includes a cathode container assembly of electrically insulating material for supporting said liquid metal cathode, said cathode container assembly being coated with a polysiloxane fluid.

## References Cited by the Examiner

## UNITED STATES PATENTS

|    |           |       |                |         |
|----|-----------|-------|----------------|---------|
| 35 | 1,364,359 | 1/21  | Edison         | 204—29  |
|    | 2,230,023 | 1/41  | Aten           | 204—21  |
|    | 2,239,144 | 4/41  | Dean et al.    | 204—10  |
| 40 | 2,386,466 | 2/40  | Hyde           | 117—232 |
|    | 2,469,888 | 5/49  | Patnode        | 260—448 |
|    | 2,950,997 | 8/60  | Halacsy        | 117—232 |
|    | 2,974,104 | 3/61  | Paine et al.   | 204—10  |
| 45 | 2,984,590 | 5/61  | Anderson       | 117—232 |
|    | 3,032,444 | 5/62  | Scadron et al. | 117—232 |
|    | 3,061,536 | 10/62 | Gruber         | 204—219 |

JOHN H. MACK, Primary Examiner.